# EUROPEAN PATENT SPECIFICATION

(11) **EP 1 422 560 B1**
(45) Date of publication and mention of the grant of the patent: **10.05.2006**
(21) Application number: 03078494.6
(22) Date of filing: 06.11.2003
(51) Int. Cl.: G03C 5/17, G03C 1/005

(54) **Radiographic film for mammography with improved processability**
Radiographischer Silberhalogenidfilm zur Mammographie mit verbesserter Verarbeitbarkeit
Film radiographique à l'halogénure d'argent ayant des caractéristiques de traitement améliorés

(30) Priority: 19.11.2002 US 299237; 19.05.2003 US 440950
(43) Date of publication of application: 26.05.2004
(73) Proprietor: EASTMAN KODAK COMPANY, Rochester, New York 14650 (US)
(72) Inventor: Dickerson, Robert E., c/o Eastman Kodak Company, Rochester New York 14650-2201 (US); Adin, Anthony, c/o Eastman Kodak Company, Rochester New York 14650-2201 (US); Beal, Richard E., c/o Eastman Kodak Company, Rochester New York 14650-2201 (US); Gingello, Anthony D., c/o Eastman Kodak Company, Rochester New York 14650-2201 (US)
(74) Representative: Haile, Helen Cynthia

(56) References cited:
- EP-A- 1 217 433
- US-A- 5 455 139
- US-A- 5 491 058

## Description

This invention is directed to radiography. In particular, it is directed to a radiographic silver halide film that provides improved medical diagnostic images of soft tissues such as in mammography and exhibits improved processing characteristics.

In conventional medical diagnostic imaging the object is to obtain an image of a patient's internal anatomy with as little X-radiation exposure as possible. The fastest imaging speeds are realized by mounting a dual-coated radiographic element between a pair of fluorescent intensifying screens for imagewise exposure. 5% or less of the exposing X-radiation passing through the patient is adsorbed directly by the latent image forming silver halide emulsion layers within the dual-coated radiographic element. Most of the X-radiation that participates in image formation is absorbed by phosphor particles within the fluorescent screens. This stimulates light emission that is more readily absorbed by the silver halide emulsion layers of the radiographic element.

While the necessity of limiting patient exposure to high levels of X-radiation was quickly appreciated, the question of patient exposure to even low levels of X-radiation emerged gradually. The separate development of soft tissue radiography, which requires much lower levels of X-radiation, can be illustrated by mammography. The first intensifying screen-film combination (imaging assembly) for mammography was introduced to the public in the early 1970's. Mammography film generally contains a single silver halide emulsion layer and is exposed by a single intensifying screen, usually interposed between the film and the source of X-radiation. Mammography utilizes low energy X-radiation, that is radiation that is predominantly of an energy level less than 40 keV.

U.S. Patent 6,033,840 (Dickerson) and U.S. Patent 6,037,112 (Dickerson) describe asymmetric imaging elements and processing methods for imaging soft tissue.

In mammography, as in many forms of soft tissue radiography, pathological features sought to be identified are often quite small and not much different in density than surrounding healthy tissue. Thus, mammography is a very difficult task in medical radiography. In addition, microcalcifications must be seen when they are as small as possible to improve detection and treatment of breast cancers. As a result, mammographic films often include relatively high amounts of silver and gelatin to maximize image sharpness when used with a single intensifying screen. The higher amounts of silver and gel may mean that the films are more difficult to process or require longer processing times.

This invention provides a solution to the noted problems with a radiographic silver halide film comprising a support having first and second major surfaces and that is capable of transmitting X-radiation,
the radiographic silver halide film having disposed on the first major support surface, one or more hydrophilic colloid layers including at least one cubic silver halide grain emulsion layer, and on the second major support surface, one or more hydrophilic colloid layers including at least one silver halide emulsion layer,
the film characterized wherein the cubic silver halide grain emulsion layer comprises cubic silver halide grains comprising from 1 to 20 mol % chloride and from 0.25 to 1.5 mol % iodide, both based on total silver in the emulsion layer, which cubic silver halide grains have an average ECD of from 0.65 to 0.8 µm.

Further, this invention provides a method of providing a black-and-white image comprising exposing a radiographic silver halide film of this invention and processing it, sequentially, with a black-and-white developing composition and a fixing composition, the processing being carried out within 90 seconds, dry-to-dry.

This invention also provides a radiographic imaging assembly comprising a radiographic silver halide film of this invention that is arranged in association with a fluorescent intensifying screen.

The present invention provides a means for providing radiographic images for mammography with a radiographic film that is readily processed using the conventional processing solutions known in the art. In addition, all other desirable sensitometric properties are maintained or improved (such as photographic speed). If desired, the amount of silver used in the films can be reduced without a significant loss in photographic speed.

These advantages are achieved by including certain cubic silver halide grains that are comprised of specific amounts of chloride, iodide, and bromide. The critical amount of iodide provides desired photographic speed and the critical amount of chloride provides desired image tone and rapid processability.

FIG. 1 is a schematic cross-sectional illustration of a radiographic silver halide film of this invention.

FIG. 2 is a schematic cross-sectional illustration of a radiographic imaging assembly of this invention comprising a radiographic silver halide film of this invention arranged in association with a single fluorescent intensifying screen in a cassette holder.

The term "contrast" as herein employed indicates the average contrast derived from a characteristic curve of a radiographic film using as a first reference point (1) a density (D₁) of 0.25 above minimum density and as a second reference point (2) a density (D₂) of 2.0 above minimum density, where contrast is ΔD (i.e. 1.75) ÷ Δlog₁₀E (log₁₀E₂ - log₁₀E₁), E₁ and E₂ being the exposure levels at the reference points (1) and (2).

The term "dual-coated" is used to define a radiographic film having silver halide emulsion layers disposed on both the front- and backsides of the support. The radiographic silver halide films of the present invention are "dual-coated."

The term "fluorescent intensifying screen" refers to a screen that absorbs X-radiation and emits light. A "prompt" emitting fluorescent intensifying screen will emit light immediately upon exposure to radiation while "storage" fluorescent screen can "store" the exposing X-radiation for emission at a later time when the screen is irradiated with other radiation (usually visible light).

The radiographic silver halide films of this invention include a flexible support having disposed on both sides thereof, one or more photographic silver halide emulsion layers and optionally one or more non-radiation sensitive hydrophilic layer(s). The silver halide emulsions in the various layers can be the same or different and can comprise mixtures of various silver halide emulsions within the requirements of this invention.

In preferred embodiments, the photographic silver halide film has at least one different silver halide emulsion on each side of the support. It is also preferred that the film has a protective overcoat (described below) over the silver halide emulsions on each side of the support.

The support is preferably a transparent film support. In its simplest possible form the transparent film support consists of a transparent film chosen to allow direct adhesion of the hydrophilic silver halide emulsion layers or other hydrophilic layers.

Polyethylene terephthalate and polyethylene naphthalate are the preferred transparent film support materials.

Preferably, the "frontside" of the support comprises one or more silver halide emulsion layers, one of which contains predominantly cubic grains (that is, more than 50 weight % of all grains). These cubic silver halide grains particularly include predominantly (at least 69 mol %) bromide, and preferably up to 89.75 mol % bromide, based on total silver in the emulsion layer. In addition, these cubic grains must have from 1 to 20 mol % chloride (preferably from 10 to 20 mol % chloride) and from 0.25 to 1.5 mol % iodide (preferably from 0.5 to 1 mol % iodide), based on total silver in the emulsion layer. The cubic silver halide grains in each silver halide emulsion unit (or silver halide emulsion layers) can be the same or different.

The amount of chloride in the cubic silver halide grains is critical to provide desired processability and image tone while the amount of iodide is critical to provide desired photographic speed. Too much chloride results in poor absorption of spectral sensitizing dyes to the grains.

It may also be desirable to employ silver halide grains that exhibit a coefficient of variation (COV) of grain ECD of less than 20% and, preferably, less than 10%. In some embodiments, it may be desirable to employ a grain population that is as highly monodisperse as can be conveniently realized.

The average silver halide grain size can vary within each emulsion layer within the film. For example, the cubic grain ECD in the radiographic silver halide film is independently and generally from 0.65 to 0.8 µm (preferably from 0.7 to 0.75 µm).

The backside ("second major support surface") of the support includes one or more silver halide emulsions, preferably at least one of which comprises predominantly tabular silver halide grains. Generally, at least 50% (and preferably at least 80%) of the silver halide grain projected area in this silver halide emulsion layer is provided by tabular grains having an average aspect ratio greater than 5, and more preferably greater than 10. The remainder of the silver halide projected area is provided by silver halide grains having one or more non-tabular morphologies. In addition, the tabular grains are predominantly (at least 90 mol %) bromide based on the total silver in the emulsion layer and includes up to 1 mol % iodide. Preferably, the tabular grains are pure silver bromide.

The backside of the radiographic silver halide film also preferably includes an antihalation layer disposed over the silver halide emulsion layer(s). This layer comprises one or more antihalation dyes or pigments dispersed on a suitable hydrophilic binder (described below). In general, such antihalation dyes or pigments are chosen to absorb whatever radiation the film is likely to be exposed to from a fluorescent intensifying screen. For example, pigments and dyes that can be used as antihalation pigments or dyes include various watersoluble, liquid crystalline, or particulate magenta or yellow filter dyes or pigments including those described for example in U.S. Patent 4,803,150 (Dickerson et al.), U.S. Patent 5,213,956 (Diehl et al.), U.S. Patent 5,399,690 (Diehl et al.), U.S. Patent 5,922,523 (Helber et al.), U.S. Patent 6,214,499 (Helber et al.), and Japanese Kokai 2-123349. One useful class of particulate antihalation dyes includes nonionic polymethine dyes such as merocyanine, oxonol, hemioxonol, styryl, and arylidene dyes as described in U.S. Patent 4,803,150 (noted above) that is incorporated herein for the definitions of those dyes. The magenta merocyanine and oxonol dyes are preferred and the oxonol dyes are most preferred.

The amounts of such dyes or pigments in the antihalation layer are generally from 1 to 3 mg/dm². A particularly useful antihalation dye is the magenta filter dye M-1 identified as follows:

The silver halide emulsion layers and other hydrophilic layers on both sides of the support of the radiographic films of this invention generally contain conventional polymer vehicles (peptizers and binders) that include both synthetically prepared and naturally occurring colloids or polymers. The most preferred polymer vehicles include gelatin or gelatin derivatives alone or in combination with other vehicles.

The silver halide emulsion layers (and other hydrophilic layers) in the radiographic films are generally hardened to various degrees using one or more conventional hardeners.

The levels of silver and polymer vehicle in the radiographic silver halide film of the present invention are not critical. In general, the total amount of silver on each side of the film is at least 10 and no more than 55 mg/dm² in one or more emulsion layers. In addition, the total coverage of polymer vehicle on each side of the film is generally at least 35 and no more than 45 mg/dm² in all of the hydrophilic layers on that side. The amounts of silver and polymer vehicle on the two sides of the support in the radiographic silver halide film can be the same or different. These amounts refer to dry weights.

The radiographic silver halide films of this invention generally include a surface protective overcoat disposed on each side of the support that typically provides physical protection of the emulsion layers. Each protective overcoat can be sub-divided into two or more individual layers.

The various coated layers of radiographic silver halide films of this invention can also contain tinting dyes to modify the image tone to transmitted or reflected light. These dyes are not decolorized during processing and may be homogeneously or heterogeneously dispersed in the various layers. Preferably, such non-bleachable tinting dyes are in a silver halide emulsion layer.

Preferred embodiments of this invention include radiographic silver halide films comprising a support having first and second major surfaces and that is capable of transmitting X-radiation,
the radiographic silver halide films having disposed on the first major support surface, one or more hydrophilic colloid layers including at least one cubic silver halide grain emulsion layer, and on the second major support surface, one or more hydrophilic colloid layers including at least one silver halide emulsion layer comprising predominantly tabular silver halide grains, and an antihalation layer,
wherein the silver halide cubic grain emulsion layer comprises predominantly cubic silver halide grains comprising from 10 to 20 mol % chloride and from 0.5 to 1.5 mol % iodide, both based on total silver in the emulsion layer, which cubic grains have an average ECD of from 0.7 to 0.75 µm, and
a protective overcoat disposed over the silver halide emulsion layers on both sides of the support.

The radiographic imaging assemblies of the present invention are composed of one radiographic silver halide film of this invention and a fluorescent intensifying screen. Usually, a single fluorescent intensifying screen is used on the "frontside" for mammography. Fluorescent intensifying screens are typically designed to absorb X-rays and to emit electromagnetic radiation having a wavelength greater than 300 nm. These screens can take any convenient form providing they meet all of the usual requirements for use in radiographic imaging.

An embodiment of the radiographic film of the present invention is illustrated in FIG. 1. On the frontside of support **10** are disposed overcoat **20**, and emulsion layer **30**. On the backside of support **10** are disposed emulsion layer **50**, antihalation layer **60**, and overcoat **70**.

FIG. 2 shows the radiographic film of FIG. 1 that is arranged in association with fluorescent intensifying screen **80** on the frontside, and both in cassette holder **90**.

Exposure and processing of the radiographic silver halide films of this invention can be undertaken in any convenient conventional manner. The exposure and processing techniques of U.S. Patent 5,021,327 and U.S. Patent 5,576,156 (both noted above) are typical for processing radiographic films. Other processing compositions (both developing and fixing compositions) are described in U.S. Patent 5,738,979 (Fitterman et al.), U.S. Patent 5,866,309 (Fitterman et al.), U.S. Patent 5,871,890 (Fitterman et al.), U.S. Patent 5,935,770 (Fitterman et al.), U.S. Patent 5,942,378 (Fitterman et al.). The processing compositions can be supplied as single- or multi-part formulations, and in concentrated form or as more diluted working strength solutions.

Exposing X-radiation is generally directed through a single fluorescent intensifying screen before it passes through the radiographic silver halide film for imaging of soft tissue such as breast tissue.

It is particularly desirable that the radiographic silver halide films of this invention be processed within 90 seconds ("dry-to-dry") and preferably within 60 seconds and at least 20 seconds, for the developing, fixing and any washing (or rinsing) steps. Such processing can be carried out in any suitable processing equipment including but not limited to, a Kodak X-OMAT^{™} RA 480 processor that can utilize Kodak Rapid Access processing chemistry. Other "rapid access processors" are described for example in U.S. Patent 3,545,971 (Barnes et al.) and EP 0 248,390A1 (Akio et al.). Preferably, the black-and-white developing compositions used during processing are free of any photographic film hardeners, such as glutaraldehyde.

Radiographic kits can include a radiographic silver halide film or imaging assembly of this invention, one or more additional fluorescent intensifying screens and/or metal screens, and/or one or more suitable processing compositions (for example black-and-white developing and fixing compositions).

The following examples are presented for illustration and the invention is not to be interpreted as limited thereby.

### Example 1:

### Radiographic Film A (Control):

Radiographic Film A was a dual-coated radiographic film with 2/3 of the silver and gelatin coated on one side of the 170 µm blue-tinted poly(ethylene terephthalate) support and the remainder coated on the opposite side of the support. The frontside had a cubic grain emulsion chemically sensitized with sulfur and gold and spectrally sensitized with Dye A-1 noted below. On the backside was an antihalation layer containing solid particle dyes to provide improved sharpness over a green-sensitized high aspect ratio tabular grain emulsion (Emulsion Layer 2). At least 50% of the total grain projected area was accounted for by tabular grains having a thickness of less than 0.3 µm and having an average aspect ratio greater than 8:1. The emulsion was monodisperse in distribution and was spectrally sensitized with 400 mg/Ag mole of anhydro-5,5-dichloro-9-ethyl-3,3'-bis(3-sulfopropyl)oxacarbocyanine hydroxide, followed by potassium iodide (300 mg/Ag mole).

Film A had the following layer arrangement and formulations on the film support:
Overcoat 1
Interlayer
Emulsion Layer 1
Support
Emulsion Layer 2
Halation Control Layer
Overcoat 2

| Overcoat 1 Formulation | Coverage (mg/dm²) |
|---|---|
| Gelatin vehicle | 4.4 |
| Methyl methacrylate matte beads | 0.35 |
| Carboacymethyl casein | 0.73 |
| Colloidal silica (LUDOX AM) | 1.1 |
| Polyacrylamide | 0.85 |
| Chrome alum | 0.032 |
| Resorcinol | 0.73 |
| Dow Corning Silicone | 0.153 |
| TRITON X-200 surfactant (Union Carbide) | 0.26 |
| LODYNE S-100 surfactant (Ciba Specialty Chem.) | 0.0097 |

| Interlayer Formulation | Coverage (mg/dm²) |
|---|---|
| Gelatin vehicle | 4.4 |

| Emulsion Layer 1 Formulation | Coverage (mg/dm²) |
|---|---|
| Cubic grain emulsion [AgBr 0.85 µm average ECD] | 40.3 |
| Gelatin vehicle | 29.6 |
| 4-Hydroxy-6-methyl-1,3,3a,7-tetraazaindene | 1 g/Ag mole |
| 1-(3-Acetamidophenyl)-5-mercaptotetrazole | 0.026 |
| Maleic acid hydrazide | 0.0076 |
| Catechol disulfonate | 0.2 |
| Glycerin | 0.22 |
| Potassium bromide | 0.13 |
| Resorcinol | 2.12 |
| Bisvinylsulfonylmethane | 0.4 % based on total gelatin in all layers on that side |

| Emulsion Layer 2 Formulation | Coverage (mg/dm²) |
|---|---|
| Tabular grain emulsion [AgBr 1.8 x 0.12 µm average size] | 10.9 |
| Gelatin vehicle | 16.4 |
| 4-Hydroxy-6-methyl-1,3,3a,7-tetraazaindene | 2.1 g/Ag mole |
| 1-(3-Acetamidophenyl)-5-mercaptotetrazole | 0.013 |
| Maleic acid hydrazide | 0.0032 |
| Catechol disulfonate | 0.2 |
| Glycerin | 0.11 |
| Potassium bromide | 0.06 |
| Resorcinol | 1.0 |
| Bisvinylsulfonylmethane | 2 % based on total gelatin in all layers on that side |

| Halation Control Layer | Coverage (mg/dm²) |
|---|---|
| Magenta filter dye M-1 (noted above) | 2.2 |
| Gelatin | 10.8 |

| Overcoat 2 Formulation | Coverage (mg/dm²) |
|---|---|
| Gelatin vehicle | 8.8 |
| Methyl methacrylate matte beads | 0.14 |
| Carboxymethyl casein | 1.25 |
| Colloidal silica (LUDOX AM) | 2.19 |
| Polyacrylamide | 1.71 |
| Chrome alum | 0.066 |
| Resorcinol | 0.15 |
| Dow Corning Silicone | 0.16 |
| TRITON X-200 surfactant | 0.26 |
| LODYNE S-100 surfactant | 0.01 |

### Radiographic Film B (Invention)

Film B was like Film A except that Emulsion Layer 1 contained a AgICIBr (0.5:15:84.5 halide mole ratio) cubic grain emulsion (0.71 µm average ECD) that was chemically sensitized with sulfur and gold and spectrally sensitized with a 340 mg/mole of Ag of Dye A-1 noted above, and Emulsion Layer 2 had the following formulation:

| Emulsion Layer 2 Formulation | Coverage (mg/dm²) |
|---|---|
| Tabular grain emulsion [AgBr 2.0 x 0.10 µm average size] | 16.1 |
| Gelatin vehicle | 10.8 |
| 4-Hydroxy-6-methyl-1,3,3a,7-tetraazaindene | 2.1 g/Ag mole |
| 1-(3-Acetamidophenyl)-5-mercaptotetrazole | 0.013 |
| Maleic acid hydrazide | 0.0032 |
| Catechol disulfonate | 0.2 |
| Glycerin | 0.11 |
| Potassium bromide | 0.06 |
| Resorcinol | 1.0 |
| Bisvinylsulfonylmethane | 2 % based on total gelatin in all layers on that side |

### Radiographic Film C (Control):

Film C was like Film A except that Emulsion Layer 1 contained AgIClBr (0.5:25:74.5 halide mole ratio) cubic grain emulsion that was chemically sensitized with sulfur and gold and spectrally sensitized with a 285 mg/mole of Ag of Dye A-1 noted above.

Samples of the films were exposed through a graduated density step tablet to a MacBeth sensitometer for 0.5 second to a 500-watt General Electric DMX projector lamp that was calibrated to 2650°K filtered with a Corning C4010 filter to simulate a green-emitting X-ray screen exposure. The film samples were processed using a processor commercially available under the trademark KODAK RP X-OMAT® film Processor M6A-N, M6B, or M35A. Development was carried out using the following black-and-white developing composition:

| | |
|---|---|
| Hydroquinone | 30 g |
| Phenidone | 1.5 g |
| Potassium hydroxide | 21 g |
| NaHCO₃ | 7.5 g |
| K₂SO₃ | 44.2 g |
| Na₂S₂O₅ | 12.6 g |
| Sodium bromide | 35 g |
| 5-Methylbenzotriazole | 0.06 g |
| Glutaraldehyde | 4.9 g |
| Water to 1 liter, pH 10 | |

The film samples were processed in each instance for less than 90 seconds. Fixing was carried out using KODAK RP X-OMAT® LO Fixer and Replenisher fixing composition (Eastman Kodak Company).

Optical densities are expressed below in terms of diffuse density as measured by a conventional X-rite Model 31 OTM densitometer that was calibrated to ANSI standard PH 2.19 and was traceable to a National Bureau of Standards calibration step tablet. The characteristic D vs. Log E curve was plotted for each radiographic film that was imaged and processed. Speed was measured at a density of 1.4 + Dₘᵢₙ. Gamma (contrast) is the slope (derivative) of the noted D vs. Log E curves.

Residual dye stain ("Dye Stain") was measured using spectrophotometric methods and calculated as the difference between density at 505 nm that corresponds to the dye absorption peak, and the density at 700 nm. This measurement corrects for differences in film fog. Measurements were done on film samples that have been processed without exposure and are nominally clear of developed silver except for fog silver. Processing was carried out in an RP X-OMAT Processor Model 480RA using KODAK RA30 Developer and KODAK LO Fixer.

The following TABLE I shows the relative sensitometry of Films A-C. Control Film A had the lowest photographic speed and contrast and the highest dye stain.

**TABLE I**

| **Film** | **Average Cubic Grain ECD (µm)** | **Grain Halide(s) (mol %)** | **Relative Speed** | **Contrast** | **Dye Stain** |
|---|---|---|---|---|---|
| A (Control) | 0.73 | Br (100) | 408 | 3.5 | 0.06 |
| B (Invention) | 0.73 | IClBr (0.5:15:84.5) | 420 | 4.3 | 0.04 |
| C (Control) | 0.71 | IClBr (0.5:25:74.5) | 416 | 4.0 | 0.03 |

### Example 2:

Further radiographic films were prepared similar to Film B of Example 1 but with various silver halide ratios and grain sizes in Emulsion Layer 1. TABLE II below provides the data for these films and the sensitometric results.

**TABLE II**

| **Film** | **Average Cubic Grain ECD (µm)** | **Halide Molar Ratio** | **Speed** | **Gamma at Density of 1.0** |
|---|---|---|---|---|
| D (Control) | 0.72 | AgBr | 400 | 4 |
| E (Control) | 0.71 | AgIBr (0.5:99.5) | 404 | 4.2 |
| F (Control) | 0.73 | AgClBr (15:85) | 405 | 4.5 |
| G (Invention) | 0.71 | AgIClBr (0.5:15:84.5) | 409 | 4.6 |
| H (Control) | 0.75 | AgIClBr (0.5:30:69.5) | 402 | 1.9 |

The data in TABLE II show that both speed and contrast increase with increasing chloride up to 30 mole % chloride. However, at that upper level, contrast and speed were severely affected. The reason for this is that it is extremely difficult to maintain good cubicity and grain monodispersity for these grain size emulsions with such high amounts of chloride. Only Film G of the present invention provided maximum speed and contrast.

### Example 3:

Several radiographic films were prepared similar to Film B of Example 1 using cubic silver halide grains with various amounts of iodide content. The chloride content for the cubic grains in each film was 13.2 mol %. The following TABLE III shows the various grain content and sensitometric results.

**TABLE III**

| **Film** | **Iodide Content (mol %)** | **Speed** | **Contrast** |
|---|---|---|---|
| I (Control) | 0 | 400 | 3.96 |
| J (Control) | 0.1 | 401 | 4.11 |
| K (Invention) | 0.3 | 402 | 4.13 |
| L (Invention) | 0.5 | 406 | 4.42 |
| M (Invention) | 1 | 405 | 4.38 |
| N (Invention) | 1.5 | 408 | 4.27 |
| O (Control) | 2 | 408 | 3.88 |

The data in TABLE III show the effect of iodide incorporation on speed and contrast. Speed increased with increased iodide levels and contrast also increased until the iodide levels reached 1.5 mol %. At higher iodide content, contrast began to drop. Films L, M, and N provided desirable speed and contrast.

## Claims

1. A radiographic silver halide film comprising a support having first and second major surfaces and that is capable of transmitting X-radiation,
said radiographic silver halide film having disposed on said first major support surface, one or more hydrophilic colloid layers including at least one cubic silver halide grain emulsion layer, and on said second major support surface, one or more hydrophilic colloid layers including at least one silver halide emulsion layer,
the film **characterized** wherein said silver halide cubic grain emulsion layer comprises cubic silver halide grains comprising from 1 to 20 mol % chloride and from 0.25 to 1.5 mol % iodide, both based on total silver in the emulsion layer, which cubic grains have an average ECD of from 0.65 to 0.8 µm.

2. The film of claim 1 wherein said cubic silver halide grains are composed of from 10 to 20 mol % chloride, based on total silver in the emulsion layer, and from 0.5 to 1.5 mol % iodide, based on total silver in the emulsion layer.

3. The film of claims 1 or 2 wherein said cubic grains have an ECD of from 0.7 to 0.75 µm.

4. The film of any of claims 1 to 3 wherein said silver halide emulsion layer on said second major support surface comprises predominantly tabular silver halide grains.

5. The film of any of claims 1 to 4 further comprising an antihalation layer disposed on said second major support surface.

6. The film of any of claims 1 to 5 wherein the amount polymer vehicle on each side of its support in a total amount of from 35 to 45 mg/dm² and a level of silver on each side of from 10 to 55 mg/dm².

7. A radiographic imaging assembly comprising the radiographic silver halide film of any of claims 1 to 6 that is arranged in association with a fluorescent intensifying screen.

8. The radiographic imaging assembly of claim 7 comprising a single fluorescent intensifying screen.

9. A method of providing a black-and-white image comprising exposing the radiographic silver halide film of any of claims 1 to 6, and processing it, sequentially, with a black-and-white developing composition and a fixing composition, the processing being carried out within 90 seconds, dry-to-dry.

10. The method of claim 9 being carried out for 60 seconds or less.

## Patentansprüche

1. Radiografischer Silberhalogenidfilm, der einen Träger mit ersten und zweiten Hauptflächen umfasst und in der Lage ist, Röntgenstrahlung zu übertragen, wobei
auf der ersten Hauptfläche des Trägers des radiografischen Silberhalogenidfilms eine oder mehrere hydrophile Kolloidschichten angeordnet sind, einschließlich mindestens einer Silberhalogenidemulsionsschicht aus kubischen Körnern, und worin auf der zweiten Hauptfläche des Trägers eine oder mehrere hydrophile Kolloidschichten angeordnet sind, einschließlich mindestens einer Silberhalogenidemulsionsschicht,
und worin der Film **dadurch gekennzeichnet ist, dass** die Silberhalogenidemulsionsschicht aus kubischen Körnern kubische Silberhalogenidkörner aus 1 bis 20 Mol.% Chlorid und zwischen 0,25 und 1,5 Mol% Iodid umfasst, beide bezogen auf das gesamte Silber in der Emulsionsschicht, wobei die kubischen Körner einen mittleren äquivalenten Kreisdurchmesser von 0,65 bis 0,8 µm aufweisen.

2. Film nach Anspruch 1, worin die kubischen Silberhalogenidkörner aus 10 bis 20 Mol.% Chlorid, bezogen auf das gesamte Silber in der Emulsionsschicht, und aus 0,5 bis 1,5 Mol.% Iodid, bezogen auf das gesamte Silber in der Emulsionsschicht, zusammengesetzt sind.

3. Film nach Anspruch 1 oder 2, worin die kubischen Körner einen äquivalenten Kreisdurchmesser von 0,7 bis 0,75 µm aufweisen.

4. Film nach einem der Ansprüche 1 bis 3, worin die Silberhalogenidemulsionsschicht auf der zweiten Hauptfläche des Trägers vorwiegend tafelförmige Silberhalogenidkörner umfasst.

5. Film nach einem der Ansprüche 1 bis 4 mit zudem einer Lichthofschutzschicht, die auf der zweiten Hauptfläche des Trägers angeordnet ist.

6. Film nach einem der Ansprüche 1 bis 5, worin die Gesamtmenge an Polymervehikeln auf jeder Seite des Trägers 35 bis 45 mg/dm² und der Silbergehalt auf jeder Seite 10 bis 55 mg/dm² beträgt.

7. Radiografische Bebilderungsanordnung aus radiografischem Silberhalogenidfilm nach einem der Ansprüche 1 bis 6, angeordnet in Wirkbeziehung mit einem fluoreszierenden Verstärkungsschirm.

8. Radiografische Bebilderungsanordnung nach Anspruch 7 mit einem einzelnen fluoreszierenden Verstärkungsschirm.

9. Verfahren zur Erzeugung eines Schwarzweißbildes, das das Belichten des radiografischen Silberhalogenidfilms nach einem der Ansprüche 1 bis 6 und das aufeinanderfolgende Verarbeiten mit einer Schwarzweiß-Entwicklungszusammensetzung und einer Fixierzusammensetzung umfasst, wobei die Verarbeitung innerhalb von 90 Sekunden vom trockenen zum trockenen Zustand durchführbar ist.

10. Verfahren nach Anspruch 9, das in maximal 60 Sekunden durchführbar ist.

## Revendications

1. Film radiographique aux halogénures d'argent comprenant un support ayant une première et une deuxième faces principales et qui est capable de transmettre les rayons X,
ledit film radiographique aux halogénures d'argent comprenant, sur ladite première face principale du support, une ou plusieurs couches de colloïde hydrophile contenant au moins une couche d'émulsion à grains cubiques d'halogénures d'argent, et, sur ladite deuxième face principale du support, une ou plusieurs couches de colloïde hydrophile contenant au moins une couche d'émulsion aux halogénures d'argent,
le film étant **caractérisé en ce que** ladite couche d'émulsion à grains cubiques d'halogénures d'argent comprend des grains cubiques d'halogénures d'argent comprenant 1 à 20 % en moles de chlorure et 0,25 à 1,5 % en moles d'iodure, par rapport à l'argent total contenu dans la couche d'émulsion, ces grains cubiques ayant un ECD moyen compris entre 0,65 et 0,8 µm.

2. Film selon la revendication 1, dans lequel lesdits grains cubiques d'halogénures d'argent sont composés de 10 à 20 % en moles de chlorure, par rapport à l'argent total contenu dans la couche d'émulsion, et 0,5 à 1,5 % en moles d'iodure, par rapport à l'argent total contenu dans la couche d'émulsion.

3. Film selon la revendication 1 ou 2, dans lequel lesdits grains cubiques ont un ECD compris entre 0,7 et 0,75 µm.

4. Film selon l'une quelconque des revendications 1 à 3, dans lequel ladite couche d'émulsion aux halogénures d'argent appliquée sur ladite deuxième face principale du support comprend principalement des grains tabulaires d'halogénures d'argent.

5. Film selon l'une quelconque des revendications 1 à 4, comprenant aussi une couche antihalo appliquée sur ladite deuxième face principale du support.

6. Film selon l'une quelconque des revendications 1 à 5, dans lequel le véhicule polymère est appliqué sur chaque face du support en une quantité totale comprise entre 35 et 45 mg/dm² et la concentration d'argent sur chaque face est comprise entre 10 et 55 mg/dm².

7. Assemblage d'imagerie radiographique comprenant le film radiographique aux halogénures d'argent selon l'une quelconque des revendications 1 à 6, associé à un écran renforçateur fluorescent.

8. Assemblage d'imagerie radiographique selon la revendication 7, comprenant un seul écran renforçateur fluorescent.

9. Procédé permettant de former une image noir et blanc comprenant l'exposition du film radiographique aux halogénures d'argent selon l'une quelconque des revendications 1 à 6, et son traitement, successivement, par un révélateur noir et blanc et par un fixateur, le traitement étant réalisé en 90 secondes maximum, sec à sec.

10. Procédé selon la revendication 9 réalisé en 60 secondes ou moins.
